

Sept. 6, 1966

S. FITTON ET AL

3,270,492

PRODUCTION OF YARNS

Filed Aug. 21, 1962

4 Sheets-Sheet 1



FIG.1.



FIG.2



FIG.3.

INVENTORS:

SYDNEY FITTON  
KISHAN VALLABHDAAS VIDHANI

By  
Burgess, Dicklage & Spring

ATTORNEYS

Sept. 6, 1966

S. FITTON ET AL

3,270,492

PRODUCTION OF YARNS

Filed Aug. 21, 1962

4 Sheets-Sheet 2



FIG. 4.



FIG. 6.



FIG. 5.

INVENTORS:

SYDNEY FITTON

KISHAN VALLABHDAS VIDHANI

By  
Burgess, Dilliger & Sprung

ATTORNEYS

Sept. 6, 1966

S. FITTON ET AL

3,270,492

PRODUCTION OF YARNS

Filed Aug. 21, 1962

4 Sheets-Sheet 3



FIG. 7.

FIG. 8.



INVENTORS:

SYDNEY FITTON, KISHAN VALLABNDAS VIDHANI

By Burgess, Dicklage & Sprung  
ATTORNEYS

Sept. 6, 1966

S. FITTON ETAL

3,270,492

PRODUCTION OF YARNS

Filed Aug. 21, 1962

4 Sheets-Sheet 4



FIG. 9.

INVENTORS

SYDNEY FITTON, NISHAN VALLABHDAAS VIDHANI

By Bingers, Dinklage & Sprung

ATTORNEYS

3,270,492

## PRODUCTION OF YARNS

Sydney Fitton, Spandon, and Kishan Vallabhdas Vidhani, Arnold, Nottingham, England, assignors to The Hosiery and Allied Trade Research Association

Filed Aug. 21, 1962, Ser. No. 218,338

Claims priority, application Great Britain, Aug. 23, 1961, 30,361/61

11 Claims. (Cl. 57—157)

This invention relates to improvements in the production of crimped continuous filament yarns, primarily made of thermoplastic material such for example as polyamides, polyesters, polyvinyl chloride, acrylonitrile, and cellulose triacetate.

These crimp yarns when produced by twisting, steam setting and untwisting, by false twisting, by stuffer box crimping, and by edge crimping, are generally characterized by their high degree of contraction from their extended state when the crimp is fully developed, and this imparts to fabrics made from the yarns, properties of high density, high extensibility and firm rigid handle, for which reason they are mainly suitable for certain types of articles such for example as men's half hose, women's stretch hose, and swimwear.

For certain other types of articles such for example as knitted outerwear, underwear, woven fabrics including for example knitted or woven dress fabrics it is desirable that the fabrics should have other characteristics such as low density, some flexibility, good draping properties and attractive handle, for which reason yarns made in the aforesaid manner are not so suitable, and instead these fabrics or articles are desirably made from particular yarns such for example as those known by the registered trademarks Saaba, Crimplene and Agilon "D," by which the fabrics or articles have the desired characteristics. These particular yarns attain the desired properties, after being crimped by general methods of twist crimping or edge crimping, by being subjected to a post treatment consisting a first operational step of stretching the crimped yarn to an extent sufficiently to straighten the yarn, a second step of allowing it to contract to a small predetermined extent, and a third operational step of heat setting it in its partially contracted form.

The desired properties possessed by most of the yarns produced in this manner are as follows:

- (a) High crimp frequency,
- (b) Low amplitude wave form crimp,
- (c) Low yarn contraction when the crimp is fully developed (the latter by heat, moisture or both), and
- (d) High effective setting temperature.

An object of the invention is to enable yarns having at least some of these desired properties to be produced in improved manner.

The invention provides a process for crimping a continuous filament yarn, primarily of thermoplastic filaments, which comprises the successive steps of applying a first molecular-modifying treatment to the yarn, discontinuing or lessening the first treatment, and crimping the yarn with the accompaniment of a second molecular-modifying treatment.

The invention also provides a process for crimping a continuous filament yarn, primarily of thermoplastic filaments, which comprises the successive steps of applying a first molecular-modifying treatment to the yarn, at least in part setting the yarn in the modified molecular form, and crimping the yarn with the accompaniment of a second molecular-modifying treatment. Conveniently both modifying treatments are of like type such as both of thermal type, or the two modifying treatments are of dissimilar types such as one of thermal

type and the other of chemical type. The process is conveniently continuous with the continuously-travelling yarn being subjected to said steps in succession. For each of the two modifying treatments the yarn is traversed through a molecular-modifying zone and between the two modifying treatments the yarn is traversed through another zone.

In the instance of thermal treatment the yarn, between the two modifying treatments, is traversed through a cooling zone, and in the instance of the chemical treatment the chemical agent is removed between the two modifying treatments.

The second modifying treatment is conveniently applied while the yarn is in a crimp-distorted condition, the crimping being conveniently effected by false twisting.

Conveniently the second modifying treatment is applied prior to passage of the yarn through a false twisting device, the twist being stopped between the two modifying treatments. The yarn may travel under predetermined stress for a first molecular-modifying treatment, under predetermined stress for a second molecular-modifying treatment, under predetermined stress for a second molecular-modifying treatment, and under predetermined stress through an intermediate zone between the two treatments.

The invention also provides a continuous process for crimping a thermoplastic yarn, which consists in withdrawing the yarn from a wound supply thereof, passing it under a first predetermined stress through a molecular-modifying zone, passing it under a second predetermined stress through a molecular-modifying zone, passing it under a third predetermined stress through an intermediate and twist stopping zone, subjecting it to a false twisting process, and winding it into a package.

The process may be applied to a flat (i.e. substantially undistorted or twistless) thermoplastic yarn which may be a mono-filament or a multi-filament yarn.

The invention further provides apparatus for crimping a continuous filament yarn, primarily of thermoplastic filaments, in a continuous process, said apparatus being of a type having means for applying a crimp distortion to the yarn accompanied by a molecular-modifying treatment, characterized by means for subjecting the running yarn to a prior treatment consisting of another molecular-modifying treatment. There are means for guiding the yarn in a path which takes it in a first treatment through molecular-modifying means, in a second treatment through molecular-modifying means and crimp-distorting means, which may be a false twisting device, and through an intermediate zone between the two modifying means. There may be twist stopping means in said intermediate zone. There may be one type of modifying means such as heater means or two types such as heater means and chemical means. Conveniently said intermediate zone is a cooling zone. The first modifying means may be a chemical swelling agent which is removed at said intermediate zone. The twist stopping means may be of the type such as tension applying devices, and nip rollers.

Conveniently the heater means is in the form of one of the following types, means providing a heated surface for contact by the yarn, radiation means, convection means, immersion means and dielectric means; where heater means are used the intermediate zone is a cooling zone provided by one of the following expedients, removing the yarn from the heating zone, or introducing cold gases, cold liquids, or cold surfaces between the two heater means; and where chemical means are used removal of the chemical swelling agent is accomplished by one of the following methods, rinsing with water, or evaporation.

The invention further provides apparatus for crimping thermoplastic yarn in a continuous process, comprising a

false twisting device, means for guiding the yarn in a path which takes it through molecular-modifying means, then through another zone and twist stopping means, next through molecular-modifying means and to the false twisting device, and means following said device for winding the treated yarn into a wound package.

The invention still further provides a crimped textile multi-filament yarn in which the filaments are made from thermoplastic synthetic material, characterized in that the yarn E.S.S.T. is between 100° C. and 130° C., the crimp rigidity is between 5% and 20%, and that, of the total yarn contraction occurring under load reducing from .1 gram/denier to zero gram/denier, at least 20% occurs substantially in the region of load reduction from .0015 gram/denier to zero gram/denier.

The above and other features of the invention set out in the appended claims are incorporated in the constructions which will now be described, as specific embodiments by way of example with reference to the accompanying drawings in which:

FIGURE 1 is a side sectional view of a first yarn treating arrangement according to the invention.

FIGURE 2 is a similar view of a second yarn treating arrangement according to the invention.

FIGURE 3 is a similar view of a third yarn treating arrangement according to the invention.

FIGURE 4 is a similar view of a fourth yarn treating arrangement according to the invention.

FIGURE 5 is a similar view of a fifth yarn treating arrangement according to the invention.

FIGURE 6 is a similar view of a sixth yarn treating arrangement according to the invention.

FIGURE 7 is a front view of apparatus for the yarn treating arrangement of FIGURE 1.

FIGURE 8 is a side sectional view of said apparatus.

FIGURE 9 is a graph illustrating the contraction characteristic of yarn made according to the invention.

In all the yarn treating arrangements hereinafter described with reference to the drawings, yarn in its flat state (i.e. substantially undistorted or twistless) travels a linear path from a supply through a molecular-modifying zone which in this instance is a heating zone, another zone which in this instance is a cooling zone, a molecular-modifying zone which in this instance is again a heating zone, and through a false twisting device to a take-up package, and provision is made for preventing the false twist present in the yarn in its second heating stage from running back into the yarn in the first heating stage.

Particularly in each illustration there is shown a package F of flat yarn, the yarn Y, rollers A feeding yarn into heating and twisting zones, a twist stopping and tension device T, molecular modifying treatment means shown as heater means H, a false twist spindle S, guide rollers G, draw-off rollers B taking yarn from the heating and twisting zones, and a yarn take-up package P. It will be realized, however, that in accordance with the present invention other molecular modifying means (not shown) may be used just as well, such as a swelling bath through which the yarn is passed.

In the modification FIGURE 1 the yarn Y is drawn from the package F of flat (i.e. substantially undistorted or twistless) yarn by feed rollers A, to run in an upwards direction through the heater H, and on leaving the heater H, the yarn Y passes through a series of guides G, G1, G2 to the twist stopper and tension device T, during which time the yarn is cooled to ambient or nearly ambient temperature. From the twist stopper and tension device T it runs, again in an upwards direction, through the heater H, and then runs via a guide G3 and the false twist spindle S through the draw-off rollers B, to the take-up package P. In travelling from the twist stopper and tension device T to the draw-off rollers B, false twist is inserted and removed.

In the second modification FIGURE 2 the yarn Y from the flat yarn package F runs initially through a twist stop-

per and tension device T', and then travels upwards through the heater H. The yarn then passes via guides G, G1, G2' to the feed rollers A during which time it is cooled to ambient or nearly ambient temperature. From the feed rollers A the yarn passes again upwards through the heater H, then through the false twist spindle S and the draw-off rollers B to the take-up package P.

In the modification FIGURE 3 two feed rollers A, A1' are employed, the yarn passing first through the feed rollers A then through the heater H, then through guides G3, G1, to the feed rollers A1' for the cooling stage and then from the feed rollers A1' again upwards through the heater H to the false twist spindle S, draw-off rollers B and take-up package P.

In the modification FIGURE 4 the yarn Y passes from the flat yarn package F, through the feed rollers A, through the heater H, and then via guides G1', G4, to the draw-off rollers B thereby by-passing the false twist spindle S on one side of it. From the draw-off rollers B

the yarn returns downwardly, by-passing the false twist spindle S on the other side of it, and via guides G5, G6 again passes through the feed rollers A and upwards again through the heater H again to the draw-off rollers B in its passage to the take-up package P., i.e. this time after passing through false twist spindle S. During passage of the yarn from the heater H via the guides G1', G4, G5, G6 back to the feed rollers A, the yarn is cooled as before.

In the modification FIGURE 5 the yarn Y passes via the feed rollers A and guides G2'', G1, first upwards outside the heater H and then downward through the heater H and out to the twist stopper and tension device T''. From the twist stopper and tension device T'' the yarn again passes upwards through the heater H and then through the false twist spindle S to the draw-off rollers B and from there to the take-up package P. The cooling of the yarn takes place during the time when the yarn leaves the heater H after its first passage therethrough and before it re-enters the heater H, i.e. where the yarn passes from the heater H through the twist stopper and tension device T'' and back to the heater H.

In the modification FIGURE 6 two separate heaters H, H1 are employed, the yarn Y passing from the flat yarn package F, through the feed rollers A and upwards through the first heater H. From this heater H the yarn Y passes further upwards through a twist stopper and tension device T''' to the second heater H1 through which it passes still further upwards through the false twisting device S and the draw-off rollers B to the take-up package P. The cooling stage is where the yarn passes from the first heater H through the twist stopper and tension device T''' to the second heater H1. The feed rollers A and the twist stopper and tension device T''' may be interchanged.

In any of the modifications the twist stopper and tension device T may be dispensed with and yarn forwarding roller means may be employed instead. The percentage difference in rates of feed of the yarn by the different rollers employed may be varied to suit requirements; by way of example, satisfactory results have been obtained by rates of feed from 3% to 5% overfeed of the flat yarn and -1% to -3% underfeed of the twisted yarn.

It will be seen that the requirements of the invention are satisfied in all the modifications by the yarn Y being first heated to molecularly modify the yarn in the flat state, (i.e. to depart from molecular alignment to a predetermined extent) and also heated in the crimped state to which it is distorted by the false twisting spindle, with an intermediate zone where the first treatment is discontinued or lessened, or the yarn is at least in part set in the modified molecular form (i.e. stabilized after the departure from molecular alignment and before heating in the crimped state).

These examples are representative of various ways of carrying the invention into effect in a continuous process. Alternatively, the process may be performed in discrete

steps, i.e. the first heat treatment described for any of the different modifications may be performed in one operation or machine, and in a separate and subsequent operation, which may be in a separate machine, the treated yarn may be subjected to any general crimp processing system.

It is to be understood that the false twisting spindle S is representative of the yarn distorting device in any general crimping system in addition to false twisting, e.g. representative of the edge in edge crimping and the stuffer box in stuffer box crimping.

The following are examples of alternative ways of applying the heat to the yarn in the two stages.

(1) Heating the flat yarn by steam heating (not as shown), and false twisting with dry heat.

(2) Heating the flat yarn and false twisting with heat using dry heat at two spaced locations (FIGURE 6).

(3) Heating the flat yarn and false twisting with heat at only one location using dry heat (FIGURES 1 to 5).

It is also to be understood that means (not shown) other than heat may be employed for obtaining equivalent molecular modification of the yarn for example as follows:

Swelling the flat yarn by soaking it in phenol or alcohol and false twisting with heat using dry heat.

It is to be further understood that yarns other than thermoplastic yarns such for example as cellulose yarns may be made by any of the methods herein described suitably modified if necessary such as in the chemical process by using a chemical appropriate to the yarn.

It will be seen that whether chemical or thermal means are adopted in the first modification of molecular structure the invention provides that either thermal or chemical means may be used in the second, i.e. that which occurs when the yarn is undergoing the crimping process. The heat setting of the yarn in either its flat state or its crimp distorted state may be by direct contact with a hot surface; by radiation or convection means; by immersion in some suitable fluid or gas; by dielectric means or by any other heating means. Cooling, after the first thermal treatment, may be accomplished by removal of the yarn from the heating zone, or by introduction of cold gases, liquids or surfaces between the two heater means. The chemical modification of the yarn in either its flat state or in its crimp distorted state may be accomplished by any suitable swelling agent appropriate to the yarn material. Removal of the swelling agent after the first stage may be accomplished by rinsing with water or by evaporation. Twist stopping means may be provided by nip rollers or by suitable arrangements of contacting surfaces such as are found in many tension applying devices, e.g. in tension gates.

In the examples of some results appertaining by way of example to polyamide and polyester yarns which will be hereinafter fully described, reference will be made to the E.S.S.T. (equivalent steam setting temperature) of the yarns which may be defined as the temperature of saturated steam which must be exceeded before the yarn begins to shrink; it is also a measure of the effective heat treatment which a yarn has received.

It should here be explained that a study of the phenomenon of heat setting in nylon 66, nylon 6 and "Terylene" yarns and fabrics has led to a residual shrinkage testing technique by which the E.S.S.T. (equivalent steam setting temperature) of any of these yarns may be determined. For full details in connection with the E.S.S.T. of yarn, see "Journal of the Textile Institute," Munden, D. L. and Slater, D., June 1959, vol. 50, T393-T403, and "British Standards Handbook" No. 11, 1963, pages 154-157.

In the crimping of thermoplastic yarns such as those mentioned above, it has been observed that the extent to which the crimping deformation imposed is retained after setting, depends on the temperature of the setting process.

Further it can be observed in the heating setting of fabrics made from such thermoplastic yarns, and in the

post treatment of such yarns as previously mentioned, that the extent to which deformation is retained after setting (or in the latter case the extent to which deformation is removed after setting) depends on the effective difference of temperature between the first and second heating setting operations.

The effectiveness of setting thermoplastic yarns by dry heat and steam being non-equivalent, it is convenient in the present examples of polyamide and polyester yarns to use the E.S.S.T. of the yarn as a measure of effective heat treatment. A study of post treated false twist and edge crimped yarns, which have found acceptance in outerwear, underwear and woven fabrics indicates that some of the desirable properties of such yarns may be listed as:

(1) The highest degree of filament separation (bulk) comparable with a low potential yarn contraction.

(2) A high crimp frequency to ensure a clear stitch structure.

(3) A high E.S.S.T. to enable such processes as fabric setting and yarn dyeing to be performed with minimum loss of yarn crimp and fabric handle.

In the normal production of a false-twist nylon 66 yarn a flat yarn with an E.S.S.T. in the region 40-50° C. is used.

The E.S.S.T. of the crimped yarn is in the region of 100-120° C. Thus the crimp is imposed with a difference in E.S.S.T. of some 60-70° C.

In the yarn process described in the invention a similar deformation is imposed with lesser difference in E.S.S.T. which may be of the order 15-30° C. and the retained deformation is much less.

The lower differential is obtained by heating the yarn before the false-twist process as distinct from the post treating method which incorporates partial development of crimp and heating setting after the false-twist process. The theory is, of course, applicable to all the aforementioned alternative methods of crimping yarn. In this respect, it should be noted that in the examples concerned with the embodiments of FIGS. 1 and 3-6 shrinkage of the yarn, as a natural result of the heat treatment before the false twist step, is in fact permitted to take place because of the overfeed of the yarn. In the example concerned with the embodiment of FIG. 2 the shrinkage is permitted to take place in spite of the underfeed of yarn because of the tension gates which allow yarn to be drawn therethrough in consequence of the shrinking action of such yarn.

Examples hereinbefore referred to of some results are as follows for nylon 66 yarns:

(a) Pre-heat treatment by steam: Separate dry heat false-twist; false-twist conditions: 80 t.p.i.: 198° C. heater plate temperature and 3% overfeed:

| E.S.S.T. in ° C. of Flat Yarn | Percent Crimp Rigidity <sup>1</sup> | E.S.S.T. in ° C. of Final Yarn |
|-------------------------------|-------------------------------------|--------------------------------|
| 90                            | 8.5                                 | 100° C. ± 5° C.                |
| 80                            | 11.5                                | -----                          |
| 70                            | 15.0                                | -----                          |

<sup>1</sup> Crimp Rigidity is the percentage yarn (hank) contraction from the extended state when measured in water at 20° C. ± 2° C. using specified weights and tensions.

(b) False-twist conditions as in (a) above.

| E.S.S.T. in ° C. of Untreated flat yarn | E.S.S.T. in ° C. of Phenol Soaked Yarn | Percent Crimp Rigidity | E.S.S.T. in ° C. of Final Yarn |
|-----------------------------------------|----------------------------------------|------------------------|--------------------------------|
| 48                                      | 70                                     | 15.0                   | 100° C. ± 5° C.                |

(c) Pre-heat treatment by dry heat: separate dry heat false-twist; false-twist conditions: 80 t.p.i.: 3% overfeed at each stage: 235° C. heater plate temperature at each stage.

| E.S.S.T. in ° C. of Flat Yarn | Percent Crimp Rigidity | E.S.S.T. in ° C. Final Yarn |
|-------------------------------|------------------------|-----------------------------|
| 103.....                      | 14                     | 124                         |

(d) Pre-heat treatment by dry heat and dry heat false-twist as continuous process. Conditions 80 t.p.i.: 1% underfeed.

| Heater Plate Temperature, ° C. | Percent Crimp Rigidity | E.S.S.T. in Final Yarn |
|--------------------------------|------------------------|------------------------|
| 200.....                       | 13.5                   | 105                    |
| 210.....                       | 15.0                   | 114                    |
| 220.....                       | 16.5                   | 119                    |
| 235.....                       | 17.5                   | 124                    |

An embodiment of the invention using the edge crimping process gave the following results:

Normal edge-crimped yarn gave a crimp rigidity of about 30% on the fully bulked yarn, i.e. yarn bulked in hank form in water at 85° C. whereas the pre-heat treated edge crimped yarn gave a crimp rigidity of about 12% on yarn similarly bulked at 85° C.

An embodiment of the invention using the stuffer box crimping system gave the following results:

Normal stuffer box crimp yarn gives a crimp rigidity of about 15% whereas the pre-heat treated stuffer box crimped yarn gave a crimp rigidity of about 10%.

Yarns produced by these methods are characterized by having a high effective yarn setting temperature, high crimp frequency, a low yarn contraction when in fabric form, and a high degree of filament separation for a given amount of yarn contraction.

Fabrics made from the yarns are consequently characterized by a very soft handle, by good recovery from extension, and a high degree of cover from a given yarn denier and stiffness of fabric construction.

These results are obtained principally by virtue of the fact that the cooling zone, or its equivalent zone, allows the yarn to become established, or stabilized, or at least in part set in the molecular modified state (of departure from molecular alignment) resulting from the first molecular modifying treatment and shrinkage by the bonding together of the molecules in a different arrangement (of departure from molecular alignment) while they are no longer in a state of flux.

Examples of nylon 66 yarns illustrating a particular contraction feature are as follows:

(a) A torque crimped textile multi-filament yarn in which the filaments are made from thermoplastic synthetic material is characterized by having an E.S.S.T. of between 100° C. and 130° C., the crimp rigidity is between 5% and 20% and that after fully developing the crimp by hot water treatment of the yarn in hank form at 50° C. the percentage of contraction of the yarn from its fully extended state (i.e. when loaded to 0.1 gram/denier) is between 40% and 55% at a load of 0.0015 gram/denier and between 65% and 80% at a load of zero grams/denier.

(b) An edge crimped textile multi-filament yarn in which the filaments are made from thermoplastic synthetic material is characterized in that the yarn E.S.S.T. is between 100° C. and 130° C., the crimp rigidity of the fully bulked yarn is between 5% and 20% and that, after fully developing the crimp by hot water treatment at 50° C. of the yarn in hank form, the percentage of contraction of the yarn from its fully extended form (i.e. when loaded to 0.1 gram/denier) lies between 17% and 23% at a load of 0.0015 gram/denier and 24% and 30% at a load of zero grams/denier.

(c) A stuffer box crimped textile multi-filament yarn in which the filaments are made from thermoplastic synthetic material is characterized in that the yarn E.S.S.T. is between 100° C. and 130° C., the crimp rigidity be-

tween 5% and 13% and that, after fully developing the crimp by hot water treatment at 50° C. of the yarn in hank form, the percentage of contraction of the yarn from its fully extended state (i.e. when loaded to 0.1 gram/denier) lies between 12% and 17% at a load of 0.0015 gram/denier and between 19% and 24% at a load of zero grams/denier.

In these examples, of the total yarn contraction occurring upon load reducing from 0.1 gram/denier to zero grams/denier, at least 20% occurs substantially in the region of load reduction from .0015 gram/denier to zero grams/denier.

A tabulated example of this in comparison with a known yarn of like type is given as follows and is illustrated in graph form in FIGURE 9:

|    | Grams/denier | Yarn according to invention (C.R. 15%) | Known false twist yarn (C.R. 32%) |
|----|--------------|----------------------------------------|-----------------------------------|
| 20 | 0.1.....     | 0                                      | 0                                 |
|    | 0.05.....    | 3                                      | 3                                 |
|    | 0.025.....   | 6                                      | 9                                 |
|    | 0.0125.....  | 12                                     | 20                                |
|    | 0.006.....   | 23                                     | 33                                |
|    | 0.003.....   | 34                                     | 49                                |
|    | 0.0015.....  | 146                                    | 260                               |
| 25 | 0.0.....     | 70                                     | 72                                |

<sup>1</sup> 24% Difference i.e. 34% of total approx.

<sup>2</sup> 12% Difference i.e. 16% of total approx.

It will be seen that whereas for the known yarn the percentage difference of contraction between the loads of .0015 gram/denier and zero grams/denier is 12% being approximately 16% of the total contraction, that for this particular yarn according to the invention is 24% being approximately 34% of the total contraction. In all other examples according to the invention of nylon 66 yarn it is found that the percentage of the total contraction under similar circumstances is at least 20%.

It is an advantage of the invention that it can be carried out on existing multi-unit crimping machines with only minor machine modifications such for examples as to yarn guides and tension devices.

A particular advantage of the use of the single heater arrangements in a multi-unit machine is that, whereas there may be variations in applied heat at the different twisting stations in the machine, it is the differential in effective heat (there being a differential by virtue of the contrasting flat and twisted states of the yarn) between the two stages at each twisting station which determines the crimp characteristics, and this differential will be substantially constant for all the twisting stations, so that the crimp will be substantially regular for all the twisting stations.

This machine adaptation is illustrated in FIGURES 7 and 8 which shows an existing multi-unit false twisting machine modified by way of example according to the modification of FIGURE 1.

Briefly there is a support frame 1, a base 2 mounting yarn packages F, brackets 3 carrying the feed rollers A, a pair of bus bars 4, 5 carrying heaters H, an angle iron support 6 for false twisting spindles S, a bracket 7 for draw-off rollers B, and bracket supports P1 for the take-up packages P. As aforesaid, the heaters H may also take the form of a different molecular modifying means (not shown), such as a container having a liquid swelling bath therein through which the yarn is passed.

An electric driving motor 8 is carried by the frame 1 and it drives a large pulley 9 driving a belt 10 one lap of which engages and drives the false twist spindles S. The belt 10 also drives another large pulley 11 which imparts drive through reduction gear means 12 to a lower spindle 13 carrying drive rollers A1 (FIGURE 1) for driving the feed rollers A. The pulley 11 (FIGURE 7) further drives, through reduction gear means 14 an upper spindle 15 carrying drive rollers B1 (FIGURE 1) for driving the feed rollers B, and the pulley 11 (FIGURE 7) still fur-

ther drives, through reduction gear means 16 an upper spindle 17 carrying rollers P2 for driving the take-up packages P.

In this example twist stopper and tension devices T are of adjustable gate type mounted on a support rod 18 which also carries the guides G2 (FIGURE 1), the other guides G, G1, G3 being mounted on the heater H.

The heater H in this example is of electric resistance type having electric resistance H2 (see FIGURE 1) with a suitable control device H3, and a thermostat H4, which together are connected to the bus bars 4, 5. The latter are connected to a suitable control unit 19 (FIGURES 1 and 7, 8) having a suitable manual control 20 and connected to mains lines M.

It will be seen that this machine is readily adapted for any of the other modifications of FIGURES 2 to 6 in a manner presenting no difficulties to those skilled in the art and therefore not being herein described in detail.

Similarly it will be understood that other modifications hereinbefore referred to may be readily carried out either on the illustrated machine or on other known machines in a manner presenting no difficulties to those skilled in the art and therefore not being herein particularly described.

What we claim is:

1. A process for crimping a thermoplastic filament, which comprises the sequential steps of submitting the filament to a shrinking treatment in which the molecular structure of the filament is modified, stabilizing the filament in its molecularly-modified condition, submitting the filament to a second molecularly-modifying treatment and physically distorting the filament to impart a crimp thereto.

2. A process for crimping a thermoplastic filament comprising the sequential steps of submitting the filament to a molecularly-modifying heat treatment, feeding the filament where it is subjected to said heat treatment at an overfeed rate permitting the filament to shrink, stabilizing the filament by cooling it in its modified condition, submitting the filament to a second molecularly-modifying treatment and physically distorting the filament to impart a crimp thereto.

3. A process for crimping a thermoplastic filament comprising the sequential steps of submitting the filament to a molecularly-modifying heat treatment, pulling the filament where it is being subjected to said heat treatment through a yarn tension device at a selected rate permitting shrinking of the filament, stabilizing the filament by cooling it in its modified condition, submitting the filament to a second molecularly-modifying treatment and physically distorting the filament to impart a crimp thereto.

4. A process for crimping a filament comprising the sequential steps of shrinking the filament in a first molecularly-modifying treatment to modify the molecular structure of the filament, stabilizing the filament in its modified condition, submitting the filament to a second molecularly-modifying treatment, physically distorting the filament by false twisting the filament, and stopping the false twist from running back into the filament in the first molecularly-modifying treatment.

5. A process for crimping a filament comprising the sequential steps of swelling the filament in a first molecularly-modifying treatment using a chemical swelling agent to modify the molecular structure of the filament and to permit shrinking thereof, stabilizing the filament in its modified condition by removing the swelling agent, submitting the filament to a second molecularly-modifying treatment to further modify the molecular structure of the filament and physically distorting the filament to impart a crimp thereto.

6. A process for crimping a nylon filament comprising the sequential steps of shrinking the filament in a first heat treatment by steam heating the filament while feeding the filament at an overfeed rate, stabilizing the filament by cooling it in its modified condition, physically distorting the filament in a second heat treatment by

dry heating the filament while imparting a false twist to the heated filament, and stopping the false twist from running back into the filament in the first heat treatment.

7. A process for crimping a nylon filament comprising the sequential steps of shrinking the filament in a first heat treatment by dry heating the filament at a selected temperature while feeding the filament at an overfeed rate, stabilizing the filament by cooling it in its modified condition, physically distorting the filament in a second heat treatment by dry heating the filament at the same temperature used in the first heat treatment while imparting a false twist to the heated filament and continuing to feed the filament at said overfeed rate, and stopping the false twist from running back into the filament in the first heat treatment.

8. A method of crimping a nylon filament in a continuous process comprising shrinking the filament in a first heat treatment by dry heating the filament while feeding the filament at a selected rate, stabilizing the filament by cooling it in its modified condition, physically distorting the filament in a second heat treatment by dry heating the filament while imparting a false twist to the heated filament, and stopping the false twist from running back into the filament from the first heat treatment.

9. A process for crimping a thermoplastic filament comprising the sequential steps of shrinking the filament in a molecularly-modifying treatment to modify the molecular structure of the filament, stabilizing the filament in its modified condition, and edge crimping the filament by passing the filament against an edge to impart a crimp to the filament.

10. A process for crimping a filament comprising the sequential steps of submitting the filament to a molecularly-modifying treatment to modify the molecular structure of the filament and to permit shrinking thereof, stabilizing the filament in its modified condition, and stuffer box crimping the filament by passing the filament through a stuffer box to impart a crimp to the filament.

11. In a process for crimping a filament comprising the sequential steps of submitting the filament to a first molecularly modifying treatment, submitting the filament to a second molecularly modifying treatment and physically distorting the filament to impart a crimp thereto, the improvement which comprises submitting the filament to first molecular modifying treatment to obtain predetermined departure from molecular alignment in the filament and stabilizing the filament in its molecularly modified condition before subjecting the filament to the second molecularly modifying treatment and crimp imparting physical distortion.

#### References Cited by the Examiner

##### UNITED STATES PATENTS

|    |           |         |                   |       |         |
|----|-----------|---------|-------------------|-------|---------|
| 55 | 2,475,922 | 7/1949  | Stockly           | ----- | 57—34   |
|    | 3,028,653 | 4/1962  | Evans             | ----- | 57—34   |
|    | 3,041,814 | 7/1962  | Held              | ----- | 57—34   |
|    | 3,067,563 | 12/1962 | Van Dijk          | ----- | 57—34   |
|    | 3,085,389 | 4/1963  | Wegener et al.    | ----- | 57—34   |
|    | 3,114,235 | 12/1963 | Griset            | ----- | 57—157  |
|    | 3,115,744 | 12/1963 | Nott              | ----- | 57—157  |
|    | 3,137,119 | 6/1964  | Crouzet           | ----- | 57—34 X |
|    | 3,142,951 | 8/1964  | Terra             | ----- | 57—34   |
|    | 3,152,435 | 10/1964 | Pittman et al.    | ----- | 57—140  |
|    | 3,154,906 | 11/1964 | Assendelft et al. | ----- | 57—34   |
|    | 3,157,022 | 11/1964 | Haynes            | ----- | 57—140  |
|    | 3,165,881 | 1/1965  | Moncuit et al.    | ----- | 57—34   |
|    | 3,167,383 | 1/1965  | Chezaud et al.    | ----- | 28—72 X |

##### FOREIGN PATENTS

70 1,260,295 3/1961 France.

MERVIN STEIN, Primary Examiner.

H. G. GARNER, D. E. WATKINS, Assistant Examiners.

75 RUSSELL C. MADER, Examiner.